

# UNITED STATES PATENT OFFICE.

EDWARD LODGE AND JAMES MORGAN EVANS, OF HUDDERSFIELD, ENGLAND, ASSIGNEES TO LODGE-EVANS NEW YORK CORPORATION, OF NEW YORK, N. Y., A CORPORATION OF NEW YORK.

## PROCESS OF DYEING.

1,181,906.

Specification of Letters Patent.

Patented May 2, 1916.

No Drawing. Original application filed December 26, 1914, Serial No. 879,210. Divided and this application filed August 12, 1915. Serial No. 45,196.

To all whom it may concern:

Be it known that we, EDWARD LODGE and JAMES MORGAN EVANS, both subjects of the King of Great Britain, and residing at 5 Huddersfield, in the county of York, England, have invented a new and useful Improvement in Processes of Dyeing, of which the following is a specification.

Our invention relates to the application 10 of sulfur dye-stuffs for dyeing animal textile fibers and fabrics (wool, hair, feathers, furs and silks) also artificial silks, and union goods composed of a mixture of animal and vegetable fibers and artificial silks 15 (i. e. animal fibers, mixed with cotton, flax, jute, rhea, ramie, china grass or hemp). The usual method of applying sulfur colors to vegetable fibers and fabrics is to reduce and dissolve the color with the aid 20 of sodium sulfid. This method is however not applicable for dyeing animal fibers or fabrics containing animal fibers, owing to the strong alkalinity of the bath dye-liquors.

25 The applicants have found that, if the sulfur colors be reduced to their leuco compounds by means of a hydrosulfite of an alkali-metal, e. g.  $\text{Na}_2\text{S}_2\text{O}_4$  or  $\text{K}_2\text{S}_2\text{O}_4$ , in presence of a normal sulfite of an alkali-metal, e. g.  $\text{Na}_2\text{SO}_3$  or  $\text{K}_2\text{SO}_3$ , and any alkali (often present in the color) removed or exchanged for the weaker alkali, ammonia, animal fibers can thereby be dyed without injury.

35 The action of the normal sulfite of an alkali-metal appears to be at least two-fold. It converts any free sulfur present in the color into thiosulfates and changes any polysulfids into thiosulfates and normal sulfids and secondly it dissolves (renders soluble) the coloring matter itself.

40 The dye-bath is most conveniently prepared by first boiling together the color and sulfite of sodium or potassium and water, then adding the hydrosulfite and stirring carefully until reduction and solution are complete. This concentrated solution of the prepared dye is added to the dye-bath containing the requisite quantity 45 of water which has previously been heated to the required temperature.

The following example may be given of

the preparation of a typical dye-bath from a commercial dyestuff, the quantities being per liter:—5 grams concentrated sulfur dye, 55 10 grams sulfite of sodium, 2 grams hydrosulfite of sodium ( $\text{Na}_2\text{S}_2\text{O}_4$ ). If the dye-stuff reacts acid, it should be made alkaline before the addition of the hydrosulfite. Or if strongly alkaline, neutral ammonium salt 60 is added to exchange caustic alkali for ammonia. Suitable ammonium salts are the chlorid, normal sulfate and acetate.

The alkalis often present in sulfid colors are sulfid of soda and caustic soda. The 65 reactions whereby they are exchanged for the weaker alkali or are removed are as follows:



As an example, wool will be worked in the dye solution at 70°-80° C. For unions 75 of cotton and wool the cotton may be dyed at a temperature up to about 40° C., on raising the temperature up to 70°-80°, the wool is then dyed. Or the order may be reversed. The addition of Glauber salt or 80 common salt assists, as is well known, exhaustion of the dye liquor.

What we claim is:—

1. A method or process of dyeing animal fibers (including furs and feathers) union 85 goods and artificial silk in any stage of manufacture, according to which sulfur colors are reduced by a hydrosulfite of an alkali-metal in the presence of a sulfite of an alkali-metal.

2. A method or process of dyeing animal fibers (including furs and feathers) union 90 goods and artificial silk in any stage of manufacture, according to which sulfur colors are reduced by a hydrosulfite of an 95 alkali-metal in the presence of a sulfite of an alkali-metal, and a neutral ammonium salt.

EDWARD LODGE.  
JAMES MORGAN EVANS.

Witnesses:

W. RAMSDEN,  
ARNOLD MELLOR.